

Feb. 15, 1966

R. W. FOWELLS ET AL

3,235,401

COATING APPARATUS AND COATING METHOD FOR MOVING WEBS

Filed March 11, 1963



Fig. 2



Fig. 3



INVENTORS  
ROBERT W. FOWELLS  
BYRON C. SHAWCROSS

J. F. Zegree  
AGENT

3,235,401

**COATING APPARATUS AND COATING METHOD  
FOR MOVING WEBS**

Robert W. Fowells, Syracuse, N.Y., and Byron C. Shawcross, Vancouver, Wash., assignors to Crown Zellerbach Corporation, San Francisco, Calif., a corporation of Nevada

Filed Mar. 11, 1963, Ser. No. 264,210  
9 Claims. (Cl. 117—102)

This invention relates to a coating apparatus and a coating method for coating of a continuous flexible web at high speeds. More particularly this invention relates to an apparatus and a coating method employing a bar means and an air knife for removal of excess of coating material on a moving web at high speeds to obtain a uniform, smooth, and high gloss coating surface.

In the past rods, scraper blades, and rolls have been used in coating operations as mechanical doctor devices to remove excess coating materials from a moving coated web. However, the finished coating surface produced by employing such doctor devices lacks uniformity in coating thickness. The use of air knife doctors to remove the excess coating and to smooth the remainder of the coating materials is well-known. While the method of smoothing a coating with air knife doctors is superior to that with the above mentioned mechanical doctor devices, many problems have become evident as high viscosities and fast coating speeds have been attempted. Air knife doctors are, for practical purposes, limited in coating speed because of turbulence in the stream of air leaving the air knife lips. This turbulence causes uneven coatings and may produce a fog with thin coating materials which then drifts to the completed coated web giving it an unsightly and grainy appearance. In addition, higher speeds require higher air pressures which in turn result in foam produced in the blow-off of many coating materials. Foam is a serious problem particularly where large amounts of coating material are continuously circulated from the blow-off to a coating container from which the coating material is applied onto a moving web.

Air turbulence problems have been attacked in many ways by attaching baffles or streamlined surface on or near the air knife lips to control the flow of air. Other air knife systems have been provided with a means to evacuate air from the area of the lips to avoid fogging of the finished coating. Even though these modifications have been improvements in the art, the basic problem of air turbulence has become increasingly evident with increased coating speeds.

In the case of air knife doctors, all excess coating material is removed by the impinging air stream. Viscous materials, however, present a problem for two reasons: First, higher air pressures are needed to doctor viscous coating materials resulting in increased turbulence in the doctored excess material which leads to uneven coatings. This problem is usually resolved by applying the coating materials at lower speeds. Secondly, higher air pressures required to doctor viscous coating materials may cause air bubbles to be entrained in the finished coating.

Accordingly, an object of this invention is to provide an apparatus and a method for coating web materials with a liquid coating material at high speeds.

Another object is to provide a method and an apparatus which employs, in combination, one or more bar means and one or more air knife doctors for uniformly applying a liquid coating material, at low or high viscosities, to a web moving at low or high speeds and obtaining a uniform, smooth, and high gloss coating surface.

Other objects and advantages of this invention will be apparent from the following description, the accompanying drawing, and the appended claims.

The present invention comprises an apparatus and a method for applying a uniform, smooth, and high gloss coating of a desired wet thickness onto a moving web including means for applying onto the web a layer of coating material; a bar means, such as a rod, for removing from the web a desired amount of excess coating material; and means for directing at the surface of the coating a stream of a gas, such as air, compatible with the composition of the coating, thereby removing any remaining excess coating material and obtaining a uniform, smooth, and high gloss coating surface.

15 A preferred embodiment of this invention will now be specifically described with reference to the accompanying drawing wherein:

FIG. 1 is a front sectional view of the preferred embodiment of the invention.

20 FIG. 2 is a side view of a bar means assembly.

FIG. 3 is a view showing portions of a wire-wound rod, such as may be used in a modification of the invention.

25 Referring now to FIGS. 1 and 2 a web 1, such as a paper web, which may move at a wide range of speeds, such as 1000 feet per minute or higher, travels around a positioning roll 3 which causes the web to contact the coating applicator roll 5. Coating material 7 of a desired composition and viscosity is brought and applied to 30 web 1 by coating applicator roll 5 to produce a coated web. Coating applicator roll 5 may be rotating in either direction with or against the direction of web travel, and at a speed equal to, greater, or slower than the speed of the web. It is preferable, however, to adjust positioning 35 roll 3 so that the area of contact between the web under tension and the roll is more than just the tangent line at the point where web 1 and applicator roll 5 meet. Applicator roll 5 is positioned so that a portion thereof is immersed in coating material 7 in a coating container, such as coating pan 15. The amount of coating material 7 applied onto web 1 is adjusted by the speed of the applicator roll and the web. The method of application of the coating material onto the web is not critical. Any known method for achieving the abovementioned purpose is satisfactory.

40 Once coating material 7 is applied onto moving web 1 by applicator roll 5 the coated web moves toward a bar means, such as rod 9, whereby any desired amount of the excess coating material may be removed from the coated web. The bar means may be a tear drop, a knife design, a taut wire or preferably a rod which may, if desired, have a smooth, indented, or wire-wound surface. FIG. 3 shows portions of a rod of the latter type, having wire 12 wound around the outer surface of bar 10.

45 Rod 9 is adjustably positioned on its support 13 so that it contacts the surface of the coated web and removes any desired portion of the excess coating material. Any distance between rod 9 and the surface of the uncoated web is governed by the desired wet thickness of the coating or the amount of coating material to be removed. However, it is preferable that rod 9 be adjusted so that it creates a tension against the web. The amount of the tension depends on the coating speed, geometry of the system, and the desired coating thickness. Rod 9 may be positioned anywhere between a point where the coating material is applied onto said web and a point P on the coated web where P is, in relation to the direction of web travel, before the first point of contact of a backing means, such as backing roll 17, with the coated web.

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335

coating pan 15 where it may again be applied onto web 1. The diameter of rod 9 may vary depending upon viscosity of coating material 7, the speed of coating, and the coating weight.

If a rod is employed for bar means 9 it may, if desired, be a rod which rotates in its channel support 11. Channel support 11 may have indentations therein for the purpose of cleaning out the rod from coating materials which may accumulate among the grooves of the indented or wire-wound rod. The rod may rotate around its axis in either direction at a speed faster or slower than the speed of the web. Drive motor 23 and reducing gear 25 may adjust the speed of the rod in a wide range, such as between 1 to 1400 feet per minute or higher.

After a desired amount of the excess coating material has been removed by rod 9 the coated web is moved on toward a coated web backing means, such as backing roll 17, where a stream of a gas, such as air, compatible with the coating composition is directed from a device, such as an air knife doctor 19, at the surface of the coating at an impingement line transverse to the direction of web travel. It is preferable to situate the air knife so that the air impingement line is formed on that portion of the coated web which is in contact with the backing roll 17. Air knife doctor 19 is positioned at a certain distance from rod 9 so that the two devices act independently and successively to control coating weight and thickness. Since one of the main objects of this invention is to apply a coating material onto a moving web at high speeds and to prevent entrainment of streaks and coating material bubbles in the finished coating, it is essential to avoid a contact of the main force of the air stream with the excess coating material being removed by rod 9. To achieve this purpose, air knife doctor 19 must be so situated that the air impingement line caused by the air knife is a sufficient distance away from and beyond rod 9 in the direction of web travel. The term "main force" of the air or gas stream denotes that force of the gas which upon contact with the excess coating material causes sufficient turbulence and air bubbles which may be entrained in the finished coating resulting in an uneven coating surface. The main force of the gas varies depending upon the gas pressure required to doctor the coated web. Accordingly, the distance between rod 9 and the air knife 19 may vary. However, air knife 19 must be positioned a sufficient distance apart from rod 9 so that the air stream from the air knife does not co-act with rod 9 at the place where the excess coating material is being removed by rod 9. In this manner the unevenness of the finished coating surface, which may be the result of close proximity of air impingement line to rod 9, is avoided. FIG. 1 illustrates a preferred positioning of air knife 19 and its distance from rod 9. The air pressure from air knife doctor 19 is adjusted so that it removes any remaining excess coating material from the web whereon a desired uniform wet coating thickness and a smooth high gloss coating surface are produced. The finished coated surface is characterized by a more uniform coating thickness and a smoother and higher gloss coating surface than that produced by either rod 9 or air knife alone. The finished coated surface is then moved on toward a dryer to be dried by any conventional means. The excess coating material removed by air knife doctor 19 falls into a blow-off container, such as pan 21, which may, if desired, continuously empty its content into coating pan 15.

One of the advantages of the present invention resides in the position of rod 9. Rod 9 may be easily adjusted for any coating thickness and readily positioned anywhere between the point where the coating material is applied onto the web and the point P. The farther the rod is from the air impingement line and the closer it is to the point of application of coating material onto the web the better coating is obtained. The rod is preferably positioned so that the excess coating material removed by the rod flows into the coating applicator pan 15. Any por-

tion or all of the excess coating material may be removed by rod 9. In most instances, it is advantageous to remove all or a major portion of the excess coating material with rod 9 and to use the air knife doctor 19 for a final coating weight adjustment and for obtaining a more uniform coating thickness and a smoother and higher gloss coating surface. Removal of a small amount of coating material by the air stream results in lower air pressures, less foam, fewer bubbles in the coated surface, and attainment of high coating speeds. If all of the excess coating material is removed by rod 9, the air knife 19 can be used to brush or smooth the coating to obtain greater smoothness and higher gloss. For example, in the case of a highly viscous coating material, removal of all or nearly all of the excess coating material reduces the doctoring load of the air knife 19 allowing higher speeds without danger of entraining air bubbles in the coating surface. Thus, increased flexibility in control of the speed of the web, coating weight, and smoothness and gloss of the coating surface are achieved by the apparatus and method of this invention.

The following examples will illustrate but in no way limit the scope of the present invention:

#### Example 1

A vinylidene-acrylic latex coating having a 60.2% solids content and a viscosity of 25 centipoises is prepared in a conventional manner. The coating apparatus employed is of the type shown in FIG. 1. A rotating rod having a diameter of 0.375 inch is used. The rod is placed adjacent to the coating applicator roll. The rotation of the rod is in the same direction as the web travel. The coating material is introduced into the coating pan as described above and applied to a moving web of paper at 800 feet per minute with an air knife pressure of 0.6 pound per square inch. 70% of excess coating material is removed by the rod. The remaining 30% excess coating material is removed by the stream of air from the air knife. The amount of foam in the air knife blow-off pan is small and a uniform, smooth and high gloss coating on the paper web is obtained.

#### Example 2

A vinylidene-acrylic latex coating having a 45% solids content and a viscosity of 25 centipoises is prepared in a conventional manner. The coating apparatus employed is of the type shown in FIG. 1. A rotating wire-wound rod having a rod diameter of 0.375 inch and a wire diameter of 0.014 inch is used. The rod is placed adjacent to the coating applicator roll. The rotation of the wire-wound rod is in the opposite direction to the web travel. The coating material is introduced into the coating pan as described above and applied to a moving web of paper at 800 feet per minute with an air knife pressure of 1.0 pound per square inch. 95% of excess coating material is removed by the rod. The remaining 5% excess coating material is removed by the stream of air from the air knife. The amount of foam in the air knife blow-off pan is nil and a uniform, smooth and high gloss coating on the paper web is obtained.

#### Example 3

A vinylidene-acrylic latex coating having a 55% solids content and a viscosity of 1000 centipoises is prepared in a conventional manner. The coating apparatus employed is of the type shown in FIG. 1. A rotating rod having a diameter of 1 inch is used. The rod is placed adjacent to the coating applicator roll. The rotation of the rod is in the opposite direction to the web travel. The coating material is introduced into the coating pan and applied to a moving web of paper at 800 feet per minute with an air knife pressure of 1.0 pound per square inch. 80% of excess coating material is removed by the rod. The remaining 20% excess coating material is removed by the stream of air from the air knife. The amount of foam in the air knife blow-off pan is very small and a uniform

smooth and high gloss coating on the paper web is obtained.

The apparatus and method of the present invention increase the capabilities of the ordinary air knife by giving higher gloss and smoother coatings at high speeds of the web. Coating quality depends primarily on its smoothness for enhanced appearance and, in the case of protective coatings, smoothness or uniformity provides the necessary coating film continuity. By the practice of the present invention, turbulence in a coating material and doctoring air are greatly reduced or eliminated which in turn reduces foam, allows higher coating speeds and higher coating material viscosities. In addition, the practice of this invention provides for a wide flexibility and control over coating variables such as coating viscosity, speed, air pressure, and coating thickness while maintaining a uniform coating.

Further advantages of the apparatus of the invention are its utility and simple construction. Any flexible moving web may be coated by the apparatus and method of this invention and many coating materials may be used, such as pigmented coatings, latex-based coatings and solvent-type coatings. This invention is not limited to coating a web on one side only. Multiple coatings can be laid on one or both surfaces of one web employing two or more bar means and air knives. The apparatus and method of the present invention may also be employed to impregnate or saturate a web with a desired material.

Having thus described the invention in preferred embodiments, we claim:

1. A method of applying a smooth and high gloss coating of a desired wet thickness of a coating material onto a moving web, which method comprises
  - (a) applying said coating material onto at least one surface of said web to produce a coated web,
  - (b) positioning a bar means between a point where said coating material is applied onto said web and a point P on said coated web where P is before the first point of contact of a backing means with the coated web,
  - (c) removing a desired amount of excess coating material by said bar means to obtain a desired coating thickness on said web,
  - (d) after so removing excess coating with said bar means, moving said web to one side of the bar means and thence upwardly in an arcuate course with said surface having the coating material thereon forming the outer convex side of the web where it moves in such course, and
  - (e) directing a stream of gas downwardly at said surface of said coated web, at an impingement line transverse to the direction of web travel, and on the outer convex side of the web where it moves in said arcuate course, to obtain a uniform, smooth, and high gloss coating surface; said impingement line being a sufficient distance away from and beyond said bar means so that the main force of said stream of gas does not come in contact with said excess coating material being removed by said bar means.

2. The method of claim 1 wherein said gas is air.

3. A method of applying a smooth and high-gloss coating of coating material onto a moving elongated web comprising

applying the coating material onto at least one surface of the web to produce a coated surface,

after the coating material has been applied, and with the surface of the web opposite its coated surface out of contact with any backing means for the web, treating the web by moving the coated surface against a physical agency that contacts the coated surface and functions by such contact to distribute the coating material on the web,

after so treating the web, moving the web laterally of such agency, and thence upwardly in an arcuate

course, with said coated surface forming the outer convex side of the web where it moves over such course, backing the web by supporting the concave side of the web where it moves over said arcuate course, and directing a stream of gas downwardly on said coated surface of the web, at an impingement line transverse to the direction of web travel, and in a region where the web is backed and the coated surface forms the convex side of the web while moving over said arcuate course, to obtain a uniform, smooth and high-gloss coating; said impingement line being a sufficient distance away from and beyond said agency so that the main force of the gas stream does not come in contact with any coating being distributed by said agency.

4. Apparatus for applying a smooth and high-gloss coating onto a moving web comprising

applicator means for applying coating material onto one surface of the web to produce a web coated over said one surface,

a backing roll spaced from the applicator means, operable to guide the web as it advances from the applicator means by supporting the surface of the web opposite the web's one surface, whereby the coated surface faces away from the backing roll on traveling over the backing roll,

said web advancing over the backing roll by progressing upwardly in an arcuate path over the outside of the roll, and said backing roll supporting the web with the web free of means contacting its said opposite surface in a reach extending between said applicator means and backing roll,

bar means for contacting the coated surface of the web in a region along said reach, operable to remove excess coating material, and

an air knife doctor for directing a stream of gas downwardly and against the coated surface of the web where the web is supported by and passes upwardly over said backing roll,

said doctor being constructed and arranged to produce an impingement line transverse to the direction of web travel, with said impingement line located a sufficient distance away from and beyond the bar means so that the main force of the stream of gas coming from the doctor does not come in contact with any excess coating material removed by said bar means.

5. The apparatus of claim 4 wherein said bar means is a rod.

6. The apparatus of claim 4 wherein said bar means is a rotating rod.

7. The apparatus of claim 4 wherein said bar means is a rod rotating in a channel support which supports the rod.

8. The apparatus of claim 4 wherein said bar means is a wire-wound rod.

9. The apparatus of claim 4 wherein said bar means is a rotating wire-wound rod.

#### References Cited by the Examiner

#### UNITED STATES PATENTS

|            |         |                 |       |           |
|------------|---------|-----------------|-------|-----------|
| Re. 22,605 | 2/1945  | Goff et al.     | ----- | 118—63 X  |
| 2,135,406  | 11/1938 | Macdonald       | ----- | 117—102 X |
| 2,334,102  | 11/1943 | Kauppi et al.   | ----- | 118—110 X |
| 2,383,964  | 9/1945  | Grupe           | ----- | 118—118 X |
| 2,632,941  | 3/1953  | Warner          | ----- | 118—118 X |
| 2,711,156  | 6/1955  | Bauling         | ----- | 117—102 X |
| 2,746,878  | 5/1956  | Rush            | ----- | 117—102 X |
| 2,995,469  | 8/1961  | Le Claire       | ----- | 117—102   |
| 3,063,868  | 11/1962 | Brandsma et al. | ----- | 117—102   |
| 3,084,663  | 4/1963  | Warner          | ----- | 118—118   |